

(No Model.)

W. R. WALTON.  
KETTLE.

No. 414,850.

Patented Nov. 12, 1889.

Fig. 1.



Fig. 2.



Witnesses

Chas. N. Smith  
J. Staib

Inventor

William R. Walton  
per Samuel W. Sorrell  
Datt

# UNITED STATES PATENT OFFICE.

WILLIAM R. WALTON, OF ANSONIA, CONNECTICUT, ASSIGNOR TO THE  
ANSONIA BRASS & COPPER COMPANY, OF SAME PLACE.

## KETTLE.

SPECIFICATION forming part of Letters Patent No. 414,850, dated November 12, 1889.

Application filed July 12, 1889. Serial No. 317,486. (No model.)

*To all whom it may concern:*

Be it known that I, WILLIAM R. WALTON, of Ansonia, in the county of New Haven and State of Connecticut, have invented an Improvement in Brass Kettles, of which the following is a specification.

In the drawings, Figure 1 is an elevation of a kettle made according to my invention; and Fig. 2 is a section, on an exaggerated scale, of a portion of the side and bottom of said kettle, *a a'* representing the side and bottom, respectively, of sheet-brass, and *b* the coating of tin applied to the interior of the kettle, the surface of which tin is smooth and planished, as before described.

In the manufacture of brass kettles it has heretofore been usual to make use of a disk of sheet-brass of the proper size and to spin the same up into the shape of the kettle by successive operations upon a form or shape, the blank kettle being annealed between one spinning operation and the next, because in the spinning operation the metal is rendered hard, and it would break if acted upon without the intermediate annealing. This machine and method of manufacturing are described in Letters Patent No. 8,589, granted to Hiram W. Hayden. In other cases the sheet-metal disk has been stamped up in dies to partially shape the same, and then the sides of the kettle-blank have been reduced by a spinning operation to take out the wrinkles and to thin the metal. Dies adapted to this object are represented in Letters Patent No. 14,887, granted May 13, 1856, to Frederick J. Seymour.

It is usual between one spinning operation and the next to pickle the article in dilute sulphuric acid to remove oxide and stains produced in the annealing operation, and any remaining acid is removed by rinsing the article in water. After the last spinning operation the metal is trimmed and a wire introduced at the rim, and in some instances the surface is finished in a lathe and the bail-ears are applied for receiving the bail. Under all circumstances it is desirable to spin the article after the last annealing operation to give the sides of the kettle the proper stiffness and elasticity, the bottom of the kettle remaining nearly the original thickness of the

sheet metal and the sides being materially reduced in thickness.

After the kettle has been otherwise finished the same has sometimes been tinned. In this case a flux composed of dilute muriate of zinc is applied to the inside of the kettle and then tin in a melted state is introduced into such kettle and adheres to the surface of the brass, and the surplus tin is poured out and the surface wiped by hand, preferably with a bunch of flax fiber, to render the tinning uniform.

It has been found in practice that the introduction of the melted tin after the last spinning operation is liable to injure the metal, because of the sudden and unequal expansion resulting from the heat of the melted tin, the metal at this stage of the process being in a hard and stiff condition, resulting from the spinning or drawing operation; hence these tinned kettles are often found to contain flaws or cracks.

I have heretofore made an application, Serial No. 309,795, filed May 6, 1889, for a patent on the method of making the kettle.

My present invention relates to the kettle itself, having the peculiarities hereinafter set forth.

In carrying out my improvement the blank kettle is manufactured in the ordinary manner up to the last annealing operation by either of the processes before described. After the last annealing operation, and before the final spinning or drawing operation, the blank kettle is carefully cleansed to remove any oxide or stain and rinsed for removing any traces of acid, and then a suitable flux—such as a dilute solution of muriate of zinc—is introduced in the inside, and then the melted tin is poured into the kettle and adheres to the inner surface thereof, and the surplus tin is poured out and the tin spread uniformly by a suitable wiper, or the tin may be applied by any of the well-known methods used in tinning metals; and I find that by applying the tinning to the metal in its annealed condition there is no risk of the metal cracking under the strain due to the expansion from the heat of the tin, and the kettle-blank at this stage is placed upon a suitable form and the final spinning or drawing operation

applied to the same for hardening the metal and rendering the same stiff and elastic, and in this operation the tinning is not in any manner injured, but, on the contrary, the tinning 5 is consolidated, smoothed, and brightened in cases where a smooth metallic chuck or form is made use of within the kettle; and the final spinning operation may be performed by rolls on the inside and on the outside of 10 the kettle, as have heretofore been made use of in the manufacture of kettles. Under all circumstances the kettle when finished by the final spinning operation is in a condition for being trimmed, wired, and 15 bailed, the tin upon the inside of the kettle being rendered smooth and uniform by the spinning operation.

The kettle manufactured by the before-described process can be distinguished from 20 tinned kettles of the ordinary make, because the tin is rendered uniform and smooth by

the last spinning operation, the form upon which the kettle is spun being smooth and polished to a greater or less extent and the tinned surface of the kettle assumes the character of tinned and planished sheet metal; hence this kettle is a new article of manufacture that can easily be distinguished in the trade from kettles made in the usual way in consequence of the peculiar character of 25 the inside surface.

I claim as my invention—

The kettle of hard-finished sheet-brass and internally tinned, the surface to the tin being smooth and planished, as a new article of 30 manufacture, substantially as set forth.

Signed by me this 1st day of July, 1889.

WILLIAM R. WALTON.

Witnesses:

WILLIAM T. LYMAN,  
I. E. STODDARD.